

# UNITED STATES PATENT OFFICE.

CARL BETHGE, OF BERLIN, GERMANY.

## FLASH-LIGHT COMPOSITION.

No. 918,818.

Specification of Letters Patent.

Patented April 20, 1909.

Application filed June 29, 1908. Serial No. 440,995.

*To all whom it may concern:*

Be it known that I, CARL BETHGE, a subject of the King of Prussia, German Emperor, and resident of 18 Schlesischestrasse, 5 Berlin, Kingdom of Prussia, German Empire, have invented a new and Improved Flash-Light Composition, of which the following is an exact specification.

The present invention relates to the production of a mixture for producing flash lights or time lights with high actinic properties for photographic and like purposes.

The novelty of the present invention consists in mixing the known combustible metals, such as magnesium, aluminum and the metals of the alkaline earths with compounds composed of thorium and acids of the heavy metals. Peroxid of thorium with an acid may also be employed with equally 20 good effect.

Compounds of the rare earths have already been employed as the oxygen carrier in the production of flash light mixtures which compounds as is known are distinguished by their strong lighting properties, thus nitrates and sulfates have hitherto been proposed. The nitrates however have not only a strong acid action but are also very hygroscopic and in consequence mixtures of 25 these nitrates with magnesium powder do not preserve their active properties. Even when preserving the ingredients separately as powders, as is usual for transport purposes, the pulverized nitrates after a short 30 time form into balls in consequence of their hygroscopic character. For this reason it is very difficult to obtain the necessary uniform mixing of the nitrates with magnesium powder. The sulfates, it is true, are not 35 hygroscopic, but naturally when in use, cause more smoke and smell and when mixed with the metals are sensitive to the moisture in the air when employed in the form of soluble salts. Further, mixtures employing 40 the sulfates are difficult to ignite. All these 45 objections are avoided by employing insoluble combinations or combinations soluble with difficulty together with the heavy metal acids. These bodies form a fine powder 50 which preserves its properties in the presence of air and which, as opposed to the nitrates, remains in powdered form either when kept apart or mixed with magnesium or other metal powder. As opposed to the 55 sulfates the mixture according to the present invention flashes with practically no smoke

or smell as only the heavy metal oxid is left behind after combustion.

The most important of the known compounds of thorium with heavy metal acids 60 for the purpose of the present invention are the chromate and the tungstate. The chromate of thorium both in the water-containing as well as in the water-free form is specially suitable for flash lights in consequence of its property of producing an 65 extraordinarily energetic flash. This property also distinguishes the chromate of thorium from the chromate of cerium which has also hitherto been proposed. When 70 mixed with magnesium powder the chromate of thorium forms an unalterable and durable flash-light mixture which flashes with extraordinary speed, produces an intensely strong light and is almost smokeless. 75 The mixtures are also in spite of their easy inflammability absolutely sure against explosion by shaking or friction and thereby satisfy all the conditions which are necessary for producing a flash light powder. 80 For producing a flash-light mixture 30 to 35 parts of magnesium powder are mixed with 70 parts of chromate of thorium.

When the heavy metal of the acid radical of the thorium compound used is tungsten 85 the corresponding tungstate of thorium produces a somewhat slower combustion and may therefore with advantage be used for "time-light" mixtures. A very good time-light mixture which is also free from smoke 90 and produces a strong light is obtained by mixing one part of magnesium powder with two parts tungstate of thorium. The proportion of the magnesium in the mixture may be altered according to the duration 95 of time for which it is desired that the powder should burn. The compounds of peroxid of thorium with acids also possess the same resistive power to the action of the air as the compounds of thorium with 100 the acids of the heavy metal described above. In addition however their higher content of active oxygen is also productive of a very effective flashing, while their proportionally small content of acid produces a 105 combustion practically without smoke and smell.

When precipitating the insoluble peroxid of thorium from solutions of thorium by means of peroxid of hydrogen it is known 110 that when ammonia is not added at the same time, a part, that is a fourth part,

of the acid of the original normal salt, separates out with the insoluble precipitate. The sulfate and the nitrate of such insoluble compounds of peroxid of thorium with acids are already well known and their production and properties have been described in detail, (see Cleve, *Bull. Soc. Chim.* (2) 43-57 and Wyrouboff and Verneuil, *Compt. Rend.* 126, 341). In consequence of this general property of the precipitates of the peroxides of thorium to hold a part of the acid it will be readily understood that other solutions of the salts of thorium may be similarly treated for the production of precipitates which have not yet been discussed in technical literature, for example the chlorate or still better for the purposes of the present invention the perchlorate on account of its smaller explosive properties.

20 As a matter of fact it is possible to obtain a gelatin like perchlorate precipitate with the same properties in a manner analogous to the process described in the literature cited above for the production of the nitrate precipitate, that is to say by adding to a solution of hydroxid of thorium in perchloric acid an excess of peroxid of hydrogen heating the same to about 60° C. and then rapidly cooling. The precipitate 25 of the perchlorate, like the nitrate precipitate, dries after sufficient washing and at ordinary temperatures to white brittle glassy pieces, which may be easily pulverized and yield a powder capable of withstanding the action of the air. This powder 30 also does not form into balls when kept for a long time and may therefore be very

rapidly and easily mixed with the magnesium powder. From the above will be seen that the compound of perchloric acid with a metal of the rare earth is particularly suited for application in the present invention as usually the normal perchlorates of the rare earths form into soapy hygroscopic masses.

40 A very good flash light mixture may be obtained by mixing one part of magnesium powder with about one part of the nitrate, sulfate or perchlorate precipitate of peroxid of thorium. For coloring the light or for prolonging the combustion or in any other way influencing the properties of the mixtures other known bodies may be added, and it will also be understood that instead of magnesium, aluminum or an alkaline earth metal may be employed.

45 I claim:—

1. A flash light composition comprising a combustible metal and a non-hygroscopic and insoluble salt of a thorium oxid, substantially as described.

50 2. A flash light composition comprising a combustible metal and a non-hygroscopic and insoluble oxidizing salt consisting of an acid of a heavy metal combined with thorium, substantially as described.

55 3. A flash light composition comprising a combustible metal and chromate of thorium.

60 In witness whereof I have hereunto set my hand in the presence of two witnesses.

65 CARL BETHGE.

Witnesses:

HENRY HASPER,  
WOLDEMAR HAUPT.